

Aug. 14, 1945.

M. E. CALLANDER

2,382,290

MANUFACTURE OF MINERAL WOOL

Filed Nov. 22, 1940

FIG. 2.



FIG. 1.

INVENTOR  
MARSHALL E. CALLANDER  
*Bruininga and Sutherland*  
ATTORNEY

## UNITED STATES PATENT OFFICE

2,382,290

## MANUFACTURE OF MINERAL WOOL

Marshall E. Callander, Columbia, Mo.

Application November 22, 1940, Serial No. 366,613

4 Claims. (Cl. 49—77.5)

This invention relates, generally, to the manufacture of mineral wool, and particularly to an improved process for manufacturing mineral wool in the form of so-called bats or mats.

In the manufacture of mineral wool, it has heretofore been customary to fiberize the molten siliceous material and project the fibers through space for a time sufficient to permit them to become solidified, before they are collected, and before they come to rest. Many efforts have been made to improve the physical characteristics of mineral wool fibers and to reduce it to various physical forms in order to better adapt it for use as insulating material; but these efforts have been largely limited by adherence to the purpose of maintaining the integrity of the individual fiberized particles.

In the manufacture of bats or mats of mineral wool, heretofore it has been customary to provide a suitable adhesive or binding substance which would render the masses thereof self sustaining.

The object of the present invention, generally stated, is to provide an improved mineral wool bat, and a process for making the same, whereby the bat will be inherently self sustaining.

Other objects of the invention will become apparent to those skilled in the art when the following description is read in connection with the accompanying drawing, in which:

Figure 1 is a view, somewhat diagrammatic in form, showing conventional mineral wool fiberizing apparatus, in connection with a collecting device constructed in accordance with one embodiment of the present invention.

Figure 2 is a detail perspective view, showing in magnified proportions a tendrillated mineral wool body, typifying the structure produced in accordance with the present invention.

In accordance with the present invention, generally stated, siliceous material of the character generally employed for the manufacture of mineral wool is reduced to a molten condition, and fiberized, as by impingement with a stream of steam or other gas projected through a nozzle in accordance with the well-known practice. The present invention is characterized, however, by the feature that the fiberized mineral wool particles are intercepted in their flight before they become completely solidified, and, as intercepted, collected and reduced to the form of bats. By thus intercepting the flight of fiberized particles of siliceous material before they are completely solidified, and collecting a group of them together, a plurality of the fibers become

autogeneously connected at their points of contact, and result in the production of a tendrillated body of mineral wool consisting of a plurality of originally discrete fibers which, however, are autogeneously connected.

Any suitable barrier may be employed for thus intercepting the flight of the fiberized particles of mineral wool, and the barrier may be maintained in the trajectory of the fiberized particles at a distance from the fiberizing mechanism such that, while the particles are fiberized before contacting the barrier, they are incompletely solidified, and in a physical condition such that upon contact with another such fiber, they will mutually solidify in autogenous relation. For example in a typical installation it was observed that when the barrier was arranged less than about four feet from the fiberizing device the particles were insufficiently formed (at the time of impact) to produce a commercially desired product, while when the distance between the barrier and the fiberizing apparatus was increased beyond eleven feet the particles had so completely solidified before impact that the autogenous connection of individual fibers did not occur to the desired extent. Hence on this instance a critical distance was established at four to eleven feet, with optimum results at about eight feet, but obviously with different minerals, at different temperatures, and under other conditions the critical distance may be less or greater.

With some batch compositions, the formed but incompletely solidified fibers resist autogenous connection with each other, apparently due to surface tension characteristics. Accordingly, in such cases, in order to minimize such inherent resistance to autogenous connection, and in any case to facilitate the autogenous connection between individually formed but yet incompletely solidified fibers, a flux of the character generally employed in soldering operations may be introduced. For example, soda ash in dry powder form may be commingled with the blast, either before or after the molten material is impinged, using for example, about one pound soda ash per ton of mineral wool. In such cases, the soda ash becomes intimately mixed with the fibers during their travel and deposition, and apparently acts to reduce the surface tension between separate fibers, with the result that autogenous connection is facilitated. Resinous compounds of the character generally employed as soldering fluxes act similarly. These may be diluted with a suitable solvent, and sprayed into the blast in a man-

ner comparable to the method of applying dust or waterproofing treatments of the character with which those skilled in the art of mineral wool manufacture are familiar.

A movable barrier may advantageously be employed, so that when the desired amount of material has been collected thereon it may be removed from the zone of the trajectory of the fiberized particles, and the collected material removed from it. Such a barrier may, for example, take the form of an endless belt, the surface of which is preferably foraminous or roughened so as to provide an anchorage for the particles of mineral wool first deposited thereon. For example, wire mesh may be employed as the barrier material.

Referring now to the drawing for an illustrative embodiment of the present invention, the usual cupola 1 is provided with a spout 2, through which the molten material is discharged as shown at 3 adjacent the face of nozzle 4. The nozzle 4 may be of any suitable type well known to those skilled in the art for fiberizing the molten siliceous material. The siliceous material is fiberized and projected in a stream 5 through an orifice 6 in a wall 7 confining a solidifying space, in accordance with the usual practice.

Arranged in the solidifying space at a distance sufficiently remote from nozzle 4 that the fiberized material has assumed a definite fiber form, but is as yet incompletely solidified, is a barrier arrangement which, in the embodiment illustrated in the drawing, consists of a pair of endless flexible members 8 and 9. The endless flexible members 8 and 9 may, for example, be formed of wire mesh. The endless barrier 8 is mounted upon a pair of rolls 10 and 11, arranged in the embodiment shown, in substantially vertical alignment. Similarly, the flexible barrier 9 is mounted upon a pair of rolls 12 and 13, which are in substantially vertical alignment with rolls 10 and 11. A suitable frame 14 is provided for supporting the respective rolls, and any suitable mechanism is provided for driving the flexible barriers so as to continuously move the same, and progressively expose different zones thereof to the stream of fiberized material projected from nozzle 4. In the embodiment shown in the drawing, the flexible barriers 8 and 9 are arranged so that their surfaces, exposed to the stream of fiberized material, are moved in converging relation, as shown by the arrows. At their most proximate points, the barriers 8 and 9 are spaced, as shown at 15, a distance substantially corresponding to the thickness of the bat to be produced. Adjacent the space 15 a suitable device for stripping the material from the barriers is provided. In the embodiment shown a doctor blade 16 and there-beyond another doctor blade 17 is provided for stripping the material from barrier 8. As shown in the drawing, blade 17 is provided with an apron 18, arranged to guide the material stripped from the barriers to a suitable conveying mechanism, such as a belt conveyor 19, of the usual type.

With the barrier mechanism positioned in a confining space at a distance from nozzle 4 such that many of the particles intercepted by the barrier mechanism are incompletely solidified at the time of interception, the respective particles accumulate upon the exposed surfaces of barriers 8 and 9, and the deposit gradually builds up as the barriers are moved, until the desired thickness of deposit at a given zone is achieved before that zone passes space 15. Obviously, if the desired thickness of deposit is not obtained in the normal

operation of the device, the velocity at which the barriers 8 and 9 are moved may be reduced; and conversely, to reduce the thickness of the deposit, the velocity of the barriers may be increased; so that accurate control of the thickness of deposit is attainable.

Obviously much of the fiberized material does not strike the barrier mechanism, as some may fall short of it; some may be projected above it; and considerable to the sides of it, in the event that the barrier does not extend for the width of the confining space. Furthermore, regardless of the position of the barrier mechanism in the confining space, some of the fiberized particles will have become completely solidified before being intercepted in their flight by the barrier mechanism. The invention therefore does not contemplate that all particles of mineral wool be collected upon the barrier before they are completely solidified, or that all particles collected upon the barrier be of the tendrillated character hereinbefore referred to. In the operation of the device shown in the drawing, the mineral wool particles will begin to collect upon barriers 8 and 9 at points such as 20 and 21, where the barriers in their movement enter the zone of the trajectory of the steady stream of fiberized particles; and as the barriers continue to move, the deposit of material accumulates until the desired thickness is attained as shown at 22 and 23. As the deposit of wool upon barriers 8 and 9 move into the bight zone 24, additional fiberized material is added, so that the two separate bodies which have been accumulated respectively upon barriers 8 and 9 become interlocked by the final deposition of fiberized particles between the accumulated bodies at, and just prior to, the point of tangence. If the point of tangence is not too remote from the nozzle 4, the last deposited particles will autogenously connect the respective bodies together. This action may in fact be facilitated by playing a flame, or by spraying an adhesive substance, upon the bodies as they converge into tangence.

By thus intercepting the flight of incompletely solidified fibers, and causing other such fibers to deposit themselves on the collected fibers, etc., the successively contacting fibers connect themselves autogenously and solidify together, forming tendrillated bodies of mineral wool such for example as that shown in Figure 2 of the drawing. The tendrillated body shown in Figure 2 is illustrative of the general character of structure obtainable in accordance with the present invention, but it is to be distinctly understood that the tendrillated body may consist of more or less autogenously connected discrete fibers than are identifiable in Figure 2. The tendrillated body shown in Figure 2 will be recognized as consisting of a plurality of originally discrete fibers, autogenously connected, but having solidified together at points such as 25, 26, 27 and 28. It is apparent that with a multiplicity of tendrillated bodies of mineral wool, such as that shown in Figure 2, distributed throughout a mass, mat, or bat, other fibers (which may have been completely solidified before the moment of deposit) will impale themselves, and interlock with the tendrillated body; and consequently it is not necessary, in order to achieve the structural advantages of the mineral wool of the present invention, that the mass, mat or bat should be wholly devoid of individually separate fibers of the ordinary type. So long as there is a liberal presence of tendrillated bodies of the general type illustrated in Figure 2 distributed throughout the mass of collected mineral

wool, the structural advantages of the present invention are achieved.

From the conveying device 19 a collected and unified mat 29, consisting of two strata 30 and 31, may be discharged to suitable mechanism for cutting and trimming to the desired shapes and sizes for employment as insulation or otherwise. The barriers may be arranged at a selected bight and the velocities properly coordinated to produce a bat of any desired thickness which is characterized by the feature that both its extended surfaces are finished in situ, so that no trimming or smoothing operation is required. Indeed such is a decided advantage whether or not the wool is characterized by the presence of tendrillated bodies as herein described.

Obviously, such mineral wool fibers as do not strike barriers 8 and 9, or such as do not remain deposited thereon, accumulate on the floor of the confining space, as shown at 32, and may be periodically removed for disposition as bulk wool.

Obviously, when and if desired, suitable lubricants, binding agents, and the like, which have heretofore been commonly employed in the art of manufacturing mineral wool bats, may be utilized in connection with the present invention to supplement the binding, strengthening, and stabilizing action of the tendrillated bodies above described in the finished masses.

From the foregoing description, it is believed that those skilled in the art will readily appreciate the advantages of the present invention, and fully perceive the improved character of the masses, bats or mats of mineral wool produced in accordance with the present invention, where the fibrous material is collected upon a barrier before the particles have completely solidified. While in the foregoing description, and in the accompanying drawing, a complete embodiment has been disclosed for the purpose of illustration, it is not to be understood that the invention is limited to the details of the foregoing disclosure; but on the contrary, that the features thereof may be applied and utilized in a variety of forms and adaptations. It is therefore to be distinctly understood that such modifications,

adaptations and the use of such individual features and combinations of features as do not depart from the spirit of this invention, are, although not specifically described herein, contemplated by and within the scope of the appended claims.

Having thus described the invention, what is claimed is:

1. In the art of making mineral wool, the process of forming coherent fluffy masses, comprising, fiberizing molten siliceous material and projecting the discrete fiberized particles in space, and collecting the particles in flight before the same have completely solidified upon a collection of similar particles.
- 10 2. In the art of making mineral wool, the process of forming coherent fluffy masses, comprising, fiberizing molten siliceous material and projecting the discrete fiberized particles in space, interposing a foraminous barrier in the trajectory of the particles in a position whereat the particles are incompletely solidified fiberized particles, and removing the material from the barrier after the particles have solidified.
- 20 3. In the art of making mineral wool, the process of forming coherent fluffy masses, comprising, fiberizing molten siliceous material and projecting the discrete fiberized particles in space, intercepting the flight of the particles before the same have completely solidified upon converging moving barriers, and removing the solidified fibers from the barriers adjacent the point of convergence.
- 25 4. In the art of making mineral wool bats, the process comprising, collecting mineral wool masses on a plurality of surfaces, and superposing the mass collected on one surface upon a mass collected on another surface and, concurrently with such superposition, interposing incompletely solidified mineral wool particles between the respective masses so that upon solidification of said interposed particles some of the fibers in one mass will be autogenously connected with some of the fibers in the other.
- 30 45

MARSHALL E. CALLANDER.